

# UNITED STATES PATENT OFFICE.

GEORGE W. CHILDS, OF NEW YORK, N. Y.

## PROCESS OF MAKING LIQUID LEATHER-DRESSING FROM TANNING LIQUORS.

No. 882,490.

Specification of Letters Patent.

Patented March 17, 1908.

Application filed September 24, 1907. Serial No. 394,303.

*To all whom it may concern:*

Be it known that I, GEORGE W. CHILDS, of New York city, in the county and State of New York, have invented a certain new and 5 useful Improvement in Processes of Making Liquid Leather-Dressings from Tanning Liquors, whereof the following is a specification.

The leather dressing produced by the process herein claimed is particularly applicable 10 to the manufacture of leather, such as sole leather, which it is desired shall attain the greatest degree of solidity possible with the necessary degree of flexibility. All processes 15 for making such leather have heretofore involved two stages:—First, the hides are subjected to the action of a liquor comprising active tannic material until combined with all of the tannin with which they are capable of combining and, second, the leather thus 20 tanned is then subjected to a loading process, which usually consists in impregnating the leather with concentrated bark extract.

The leather dressing hereinafter described is adapted to impregnate hides contemporaneously 25 with an active tannic material and with an inert (non-tannic) loading material so that the required effect is produced in much less time than if said materials were applied successively as heretofore, and, said 30 inert loading material being less costly than the active tannic material heretofore employed for loading purposes, the cost of the dressed leather is correspondingly less than heretofore. Said dressing is conveniently 35 formed by mixing sapped or exhausted tanning liquor containing a high percentage of inert solid matter, with fresh tanning liquor containing active tannic material, and then concentrating the mixture until it is from 40 1.05 to 1.3 specific gravity.

I prefer to employ waste tanning liquors which are devoid of the acid or alkaline impurities which are usually found in such liquors. For instance, if the waste liquor is 45 from an acid tanning yard, and contains sulfuric or other non-volatile mineral acid, it may be neutralized by the addition of alkali, for instance sodium hydrate, or potassium hydrate, or, the acids may be precipitated as salts by the addition of bases forming insoluble compounds with the acids; for instance, barium chlorid. If the waste liquor is from a non-acid yard and contains lime or lime compounds, such impurities

may be precipitated by the addition of chemicals forming insoluble compounds with lime; for instance, ammonium oxalate, sodium phosphate, sodium fluorid, or carbon di- 55 oxid gas may be employed to effect such precipitation. On the other hand, if the waste liquor does not contain the mineral impurities aforesaid, but contains volatile impurities, for instance, volatile acids, such impurities may be eliminated by heating the liquor. The waste liquor may be mixed 60 with fresh tanning liquor or bark extract and then concentrated, conveniently by heating *in vacuo*, until it is from 1.05 to 1.3 specific gravity. It may be observed that if said dressing were of less specific gravity, there 65 would not be sufficient solid residue thereof when the leather is dried to obtain the result desired. Moreover, if said dressing were of a greater specific gravity, it would not be absorbed by the leather. 70

Said dressing may be utilized as follows:— Hides which have been treated in vats with any suitable tanning solution until they are colored through, are placed in a rotary drum, and said dressing, preferably heated, introduced to said drum, conveniently through a hollow axle or trunnion thereof, and the revolution of said drum continued until said dressing is absorbed by the hides. The hide substance having then combined with all of the tannin with which it will combine, and the pores of the leather being filled with said dressing; when dried, the residue of the dressing in the leather not only renders the latter 85 more solid than if it had not been impregnated with said dressing, but also adds materially to its final weight. Leather treated 90 as last described, may then be bleached oiled, dried, dampened and rolled in the usual manner. 95

A process for treating waste tanning liquor containing mineral acid impurities, as above contemplated, forms the subject matter of my application Serial #317,141, filed May 16, 1906, for Letters Patent of the United States, 100 and, a process for treating leather with concentrated waste tanning liquor, as above contemplated, forms the subject matter of my application Serial #327,029, filed July 20, 1906, for Letters Patent of the United States. 105

I do not desire to limit myself to all of the details of procedure above enumerated, as various modifications may be made therein

without departing from the essential features of my invention, as defined in the appended claims.

I claim:—

- 5 1. The process of making leather dressing which consists in mixing waste tanning liquor with active tanning material and concentrating the mixture until it is from 1.05 to 1.3 specific gravity.
- 10 2. The process of making leather dressing from tanning liquors, which consists in mix-

ing waste tanning liquor with active tanning liquor and concentrating the mixture until it is of from 1.05 to 1.3 specific gravity.

In testimony whereof, I have hereunto <sup>15</sup> signed my name at New York city, N. Y. this the thirteenth day of September 1907.

GEORGE W. CHILDS.

Witnesses:

HENRY W. HEALY,  
JNO. P. ANDERSON.